

## COMPOSITIONS OF MATTER

Hugh B. Hix, Wilmington, Del., assignor to E. I. du Pont de Nemours and Company, Wilmington, Del., a corporation of Delaware

No Drawing. Application August 1, 1956  
Serial No. 601,341

2 Claims. (Cl. 75—174)

This invention relates to niobium-base alloys, and more particularly to niobium-base alloys containing titanium and at least one other element of the group comprising aluminum, beryllium, carbon, cobalt, iron, manganese, molybdenum, nickel, silicon, tantalum, tungsten, vanadium and zirconium.

Superior, workable alloys which possess strength and oxidation resistance at high temperature are used as materials of construction in all types of technical and industrial equipment. The development of more advanced nuclear reactors and gas turbines is dependent upon the availability of such alloys. Furthermore, there is a need for better, high temperature alloys in the construction of dies for high temperature working of metals and the construction of chemical reactors, oil refining equipment, and the like. A combination of workability, high temperature strength, and high temperature corrosion resistance in an alloy has proved difficult to achieve, and considerable time and effort have been devoted to the search for such metals.

It has now been found that workable alloys possessing unusually high corrosion resistance and strength at temperatures above 1100° C. can be produced by alloying titanium and niobium and specified added elements in the amounts set forth herein.

It is, therefore, an object of this invention to provide for the production of niobium-base alloys which are particularly resistant to high temperature oxidation. Another object of my invention is to provide niobium-base alloys which are responsive to heat-treatment. Another object of my invention is to produce niobium-base alloys to which a film of metal oxide will firmly adhere when the alloy is heated to relatively high temperatures and cooled. Other objects and advantages of the present invention will be apparent in view of the following detailed descriptions thereof.

The alloys of this invention comprise compositions containing about 1-30% by weight of titanium, about 0-10% by weight of aluminum, about 0-5% by weight of beryllium, about 0-2% by weight of carbon, about 0-5% by weight of cobalt, about 0-10% by weight of iron, about 0-10% by weight of manganese, about 0-20% by weight of molybdenum, about 0-5% by weight of nickel, about 0-2% by weight of silicon, about 0-20% by weight of tantalum, about 0-5% by weight of tungsten, about 0-10% by weight of vanadium and about 0-20% by weight of zirconium, the sum total of Al, Be, C, Co, Fe, Mn, Mo, Si, Ni, Ta, W, V and Zr ranging from about 1-20% by weight, the balance being essentially niobium.

In a more preferred embodiment the alloys of this invention comprise about 5-25% by weight of titanium, about 0-5% by weight of aluminum, about 0-5% by weight of nickel, about 0-5% by weight of iron, about 0-7% by weight of molybdenum, the sum total of Al, Ni, Fe and Mo being about 4-20% by weight, the balance being essentially niobium.

The methods for preparing alloys of this invention follow conventional metal melting and remelting tech-

niques using inert conditions. Measured amounts of the individual metal constituents are melted together, solidified and remelted until homogeneity is obtained. The final melt is then allowed to cool and solidify into a desired shape. The case material thus obtained is of a workable metal with strength and oxidation resistance at high temperatures, and it is suitable as a material of construction in high temperature equipment. Any of a number of types of melting equipment may be used to prepare these new alloys. In the specific examples which appear later in this specification, an arc melting furnace of the type described by W. Kroll in "Transactions of the Electrochemical Society," vol. 78, pp. 35-47, 1940, was used. This furnace has an integral, water-cooled copper crucible in which the charge may be melted and solidified. The charge of metal constituents for this furnace may be in any convenient form, e.g., powder, shot, wire, sponge, etc. A consumable arc electrode furnace as described in U. S. Patent 2,640,860 is another apparatus which would prove suitable. Also, one could use a combination of non-consumable and consumable electrodes in a double melt furnace such as is described in U. S. Patent 2,541,764. A continuous feed furnace such as is described in U. S. P. B. Report 111,083 would also prepare the alloys. Furthermore, melting could be accomplished by inductively heating the charge in a suitable crucible. Regardless of the melting apparatus used, care should be exercised to protect the molten metals from the normal atmosphere since contamination of the alloy by oxygen, nitrogen, etc., is to be avoided. To provide protection against contamination, the melting should be carried out under inert conditions, such as an atmosphere of argon or a protective slag or a combination of a protective slag and a controlled atmosphere. The practice of using an inert atmosphere such as argon, helium, etc., when melting metals, is well known in the art.

The following examples are presented to illustrate the preparation of specific alloys of this invention and the outstanding properties of these alloys. These examples are illustrative only and are not to be construed as limiting the invention. All percents set forth in the ensuing examples refer to percents by weight.

## Example I

A uniform melt containing 23% titanium, 4% nickel, 3% aluminum and 7% niobium, was prepared by melting the elemental metals together and then alternately solidifying and remelting the alloy composition six times. The melting apparatus was an arc melting furnace having an integral, water-cooled copper crucible, as described by Kroll in the "Transactions of the Electrochemical Society" publication referred to above. A portion of the melt was poured into a water-cooled copper mold having a cylindrical cavity  $\frac{3}{4}$ " in diameter and 2" deep. During the above-described operations an atmosphere of helium was maintained above the metals to prevent contamination. The casting recovered from the mold was forged and machined into a nozzle for spraying molten salts, such as  $MgCl_2$ , in chemical processes.

The alloy composition of this example was tested for high temperature oxidation resistance by the following procedure:

A weighed sample of the alloy (in a porcelain crucible which is slotted to insure adequate access of air to the ingot) is placed in a "Globar" furnace and exposed for at least 16 hours at 1000° C. to an air purge of 2 cu. ft./min. After exposure, the sample is cooled and weighed, and the amount of oxidation is determined as the percent weight gain in the sample.

Under these conditions the alloy showed a weight gain of 1.5%. Unalloyed niobium shows a weight gain of 20% under the same conditions.

*Example II*

An alloy containing 20% titanium, 75% niobium, 3% aluminum and 2% cobalt was prepared according to the following procedure: The individual metal constituents were melted together in the furnace used in Example I using a helium atmosphere. The helium atmosphere was maintained and the alloy composition was alternately remelted and solidified six times, whereupon a homogeneous ingot was obtained. The weight gain according to the test described in Example I was 2.5%.

*Example III*

Using the procedure of Example II, an alloy of the following composition was prepared: 20% titanium, 10% aluminum and 70% niobium. The weight gain according to the test described in Example I was 1.7%.

*Example IV*

Using the procedure of Example II, an alloy of the following composition was prepared: 80% niobium, 17% titanium, 1% tungsten, 0.5% beryllium, 1.5% tantalum. The weight gain according to the test described in Example I was 2.0%.

*Example V*

Using the procedure of Example II, an alloy of the following composition was prepared: 55% niobium, 29% titanium, 5% manganese, 10% molybdenum, 1% aluminum. The weight gain according to the test described in Example I was 1.3%.

*Example VI*

Using the procedure of Example II, an alloy of the following composition was prepared: 78% niobium, 13.5% titanium, 3% aluminum, 2.5% iron, 3% molybdenum. The weight gain according to the test described in Example I was 2.2%.

*Example VII*

Using the procedure of Example II, an alloy of the following composition was prepared: 70% niobium, 16% titanium, 4% aluminum, 2% iron, 5% molybdenum, 3% beryllium. The weight gain according to the test described in Example I was 1.8%.

*Example VIII*

Using the procedure of Example II, an alloy of the following composition was prepared: 80% niobium, 15% titanium, 1% silicon, 4% aluminum. The weight gain according to the test described in Example I was 2.0%.

*Example IX*

Using the procedure of Example II, an alloy of the following composition was prepared: 65% niobium, 15% titanium, 15% molybdenum, 5% aluminum. The weight gain according to the test described in Example I was 2.2%.

*Example X*

Using the procedure of Example II, an alloy of the following composition was prepared: 90% niobium, 7% titanium, 3% aluminum. The weight gain according to the test described in Example I was 2.5%.

*Example XI*

Using the procedure of Example II, an alloy of the following composition was prepared: 75% niobium, 5% titanium, 15% zirconium, 3% aluminum, 1% vanadium, 1% tantalum. The weight gain according to the test described in Example I was 2.3%.

*Example XII*

Using the procedure of Example II, an alloy of the following composition was prepared: 80% niobium, 5% titanium, 2.5% iron, 2.5% molybdenum, 10% aluminum. The weight gain according to the test described in Example I was 2.1%.

*Example XIII*

Using the procedure of Example II, an alloy of the following composition was prepared: 70% niobium, 10% titanium, 8% vanadium, 6% molybdenum, 6% aluminum. 5 The weight gain according to the test described in Example I was 1.5%.

*Example XIV*

Using the procedure of Example II, an alloy of the following composition was prepared: 70% niobium, 15% titanium, 3.5% iron, 4.5% aluminum, 7% molybdenum. 10 The weight gain according to the test described in Example I was 1.9%.

Although it is preferable to use metals which are of a high purity, a fair amount of variance in purity can be tolerated before product quality suffers appreciably. The alloys of the working examples are made from commercially available metals containing less than 1% incidental impurities. Commercial niobium nearly always contains tantalum (usually in amounts up to 5%) which is hard to detect and very difficult to separate. Therefore, the niobium used in the specific examples no doubt contained tantalum which is reported as niobium rather than as an incidental impurity. In addition to the tantalum which is present in commercial niobium, this invention contemplates the addition of tantalum to the alloy composition in amounts up to 20%. Those skilled in the art are readily aware of the presence of incidental impurities in commercial metals and of the presence of tantalum in commercial niobium, and these facts should be taken into consideration when practicing the invention and construing the claims.

The alloys of this invention have the advantages of strength at high temperatures, ease of working, and resistance to corrosion. In addition to these advantageous properties, these alloys are superior base metals since they have resistance to oxidative deterioration at high temperatures. This property has been particularly deficient in niobium metal. These alloys are suitable for many diverse applications. Among these are the construction of pieces of equipment which must operate above 800° C.

Particular stress has been laid upon the use of these alloys in high temperature equipment, such as jet engine parts, nuclear reactor and gas turbine parts because of 45 their outstanding properties. However, it should be emphasized that its use is not limited to high temperature conditions or to any piece of equipment described herein.

Since it is obvious that many changes and modifications can be made in the above-described details without departing from the nature and spirit of the invention, it is to be understood that the invention is not to be limited to 50 said details except as set forth in the appended claims.

This case is a continuation in part of my copending application Serial No. 550,764, filed December 2, 1955.

*I claim:*

1. A niobium base alloy comprising about 1-30% by weight of titanium, about 0-10% by weight of aluminum, about 0-5% by weight of beryllium, about 0-2% by weight of carbon, about 0-5% by weight of cobalt, about 60 0-10% by weight of iron, about 0-10% by weight of manganese, about 0-20% by weight of molybdenum, about 0-5% by weight of nickel, about 0-2% by weight of silicon, about 0-20% by weight of tantalum, about 0-5% by weight of tungsten, about 0-10% by weight of vanadium, and about 0-20% by weight of zirconium, the sum total of Al, Be, C, Co, Fe, Mn, Mo, Si, Ni, Ta, W, V and Zr ranging from about 1-20% by weight, the balance being essentially niobium.

2. A niobium base alloy comprising about 5-25% by weight of titanium, about 0-5% by weight of aluminum, about 0-5% by weight of nickel, about 0-5% by weight of iron, about 0-7% by weight of molybdenum, the sum total of Al, Ni, Fe and Mo being about 4-20% by weight, the balance being essentially niobium.